

## UNITED STATES PATENT OFFICE.

FRIEDRICH WILHELM WEBER, OF HACKENSACK, NEW JERSEY, ASSIGNOR TO MAYWOOD CHEMICAL WORKS, OF MAYWOOD, NEW JERSEY, A CORPORATION OF NEW JERSEY.

## METHOD OF TREATING ANIMAL TISSUE AND PRODUCTS OBTAINED THEREFROM.

No Drawing. Application filed April 4, 1924, Serial No. 704,282. Renewed August 6, 1926.

This invention relates to certain products obtained from animal tissue, for instance animal hides in their dehaired state as well as with their natural hair growth thereon; 5 it furthermore relates to a tanning process applying solutions of compounds of the rare earth metals as a tanning agent.

It is an object of the invention to provide a process furnishing a leather of superior 10 whiteness and of unusual lasting properties.

It is another object of the invention to provide a process by which a better quality of leather can be produced with considerable economical advantages.

15 It is a further object of the invention to provide a process which dispenses with the alum on account of its well known shortcomings and furnishes at a low cost an even better leather than that obtained with alum.

20 In the present art of tanning the utilization of alum plays a great part though it has considerable shortcomings because it contains a high amount of acid as is illustrated by its formula  $Al_2(SO_4)_3 + 24H_2O$ , which

25 shows that in view of the low atomic weight of aluminum the percentage of acid in the molecule of alum is enormously high; though the alum is classed among the low priced heavy chemicals its cost for the pur-

30 poses of the manufacture of leather is by no means low as the alum must be deprived at the tannery of its iron content before it can be applied for tanning; also the considerable freight charges its great amount of

35 water of crystallization are a burdensome and useless expense. The unusually high proportion of acid in the alum requires a considerable amount of alkali to neutralize it; it is also possible that leather produced by a

40 tanning process, applying alum as a tanning agent, will retain sulfuric acid within its intercellular spaces so that it is absorbed by the tissue and in the course of time will act on the leather and will render it brittle; such

45 leather will then easily crumble to pieces on handling it.

Notwithstanding such considerable shortcomings alum is yet applied on a large scale for tanning purposes because it has been 50 found very difficult to find a proper substitute for same.

I have now found that the compounds of the rare earth metals readily act as tanning agents as far as the quality of the leather and the cost of its production is concerned. 55 Notwithstanding the relatively high price which the compounds of the rare earth metals usually obtain on the market on account of the high price of the raw material, the leather obtained by my new tanning 60 process based on the application of the compounds of the rare earth metals is produced at such a low cost that it can successfully compete with the leather produced by any other process. It is probably due to the low 65 solubility of the sulfates of the rare earth metals and of the double salts formed by same, that the rare earth metals were not considered as suitable tanning agents; another reason was also that the rare earth 70 metal compounds offered on the market for other purposes were actually too high in price to admit even of the thought of using them as tanning agents. Nor did the other sources of raw material, from which such 75 compounds could be drawn, present themselves in such form as to suggest the proposition of rendering them available for tanning purposes, but the economical situation in the manufacture of chemicals for incandescent gas light has greatly changed with the enormous progress of the electric light and confronts the manufacturers of such chemicals with new problems. In my efforts of extracting the values contained in 80 monazite sand and in the residue obtained in the manufacture of compounds for impregnating the mantles for incandescent gas light I found that the rare earth metal compounds derived from these materials acted 85 as excellent tanning agents in every respect and in some points are even superior to any other such agent as will be more thoroughly pointed out hereinafter.

For the better understanding of my invention I refer to the fact that in the tanning with alum a certain amount of sodium chloride is added; practical tanners maintain that on account of its hygroscopicity the sodium chloride in the animal tissue later on softens the same after it has passed the tanning process. On the other side it is claimed 95 100

that the addition of sodium chloride to a tanning liquor containing aluminum sulfate causes a double decomposition to take place which results in the formation of



of which the  $AlCl_3$  is supposed to act as the real tanning agent. The contention of both parties are refuted by the experiments of 10 Knapp, (Die Natur und das Wesen der Gerberei-Chemie, 1858; Ueber Gerberei & Leder, Dingler's Polytechn. Journal, vol. 181, pg. 311; Rogers, Practical Tanning, 1923, Carey, Baird & Co., New York; Brit. 15 Pat. 2716—D. R. P. 444 & 10.518) said experiments proving that a solution of  $AlCl_3$  does not act differently upon albumen from a solution of aluminum sulfate and that in both cases the desired coagulate can only be 20 obtained upon the addition of sodium chloride.

I have now found that upon the addition of a concentrated sodium chloride solution, for instance a 10% solution, to a 5% solution of the basic acetates of a mixture of the rare earth metals a strong smell of acetic acid is noticed as soon as the animal tissue is introduced into the combined solutions, but no coagulation takes place. The animal 25 tissue, or hide, however, is thoroughly penetrated and a deposition of rare earth metal compounds practically free of acid takes place in the intercellular spaces; while the hide is dried, acetic acid is still evaporating 30 and the leather finally obtained appears perfectly white.

I have furthermore found that I can sterilize the hides by acting on the same with the salts of the rare earth metals mentioned above. This is important because the sterilization of the hides prevents their destruction by the putrefaction caused by the organic matter, like flesh particles, blood etc., adhering to the hides; on the other side 40 it is very important that this sterilization be effected with materials which are not detrimental to the hides nor to the people who are using the manufactures made from the sterilized leather. For instance formaldehyde is very effective in preventing putrefaction, but it is highly injurious to the leather as well as to the wearer of the leather product.

I have now found that I can accomplish 55 the sterilization of the hides most satisfactorily in every respect by the action of the rare earth metal salts referred to and applied to the leather by the processes described above. I have especially found that 60 leathers tanned by these processes are distinguished by being proof to mildew; this is strikingly shown by the following test which consisted in moistening leather, having been tanned by any of the above processes, with water and subsequently drying it

in an open pan at a temperature slightly above that of the atmosphere, and continuing these operations alternately for 22 weeks without generating even the slightest trace of mildew. It is obvious therefore, 70 that leather, obtained by any of my processes described above, is especially suitable for leather goods intended to be used in tropic climates where the heat and the enormous amount of moisture in the air combine to thoroughly cover goods, made from leather tanned by other than my processes, in a few days with a layer of mildew.

This tannage may also be obtained in the 75 following manner:

The best socalled French kid leather, famous for its whiteness and softness as well as for its elasticity, was up to now thought possible only by working the hides in a drum with a semiliquid paste of a mixture of 80 aluminum sulfate with wheat flour, egg-yolk sodium chloride and warm water at the temperature of approximately 37 deg. C. The aluminum sulfate was known to have the disadvantage already mentioned above 85 and many efforts to substitute said aluminum sulfate were always accompanied by a negative result. It was especially the traces of acid retained by the animal tissue which were felt very keenly because such leather 90 had a tendency to be brittle and occasionally displayed rust spots which were caused by the retained acid when the leather came into contact with iron, the exudations of the animal tissue, including valerianic and butyric 95 acid, in the presence of sodium chloride 100 favoring the formation of such rust spots, or eventually spots caused by other metals.

In my new tanning process I can produce a leather which is superior to the socalled French kid leather by treating, preferably at 37 deg. C., the prepared hides with a solution of the acetates of the rare earth metals to which the usual quantity of egg-yolk, wheat flour and sodium chloride has 105 been added. As the applied compounds of the rare earth metals are free of sulfuric acid as well as of the slightest trace of iron, the leather obtained by my new process is of 110 superior softness and elasticity as well as of 115 permanent whiteness.

This result was rather unexpected as experiments with salts containing a proportionately great quantity of cerous chloride,  $CeCl_3$ , yielded an unsatisfactory leather 120 owing to its yellow color and its poor tanning. From a long line of experiments I have found that the cause of this is the continuous alternate change of the cerous oxide into ceri-oxide and vice versa, resulting in 125 the destruction of the skin. This undesirable feature is, however, entirely avoided by the application of the acetates of the rare earth metals; I have observed in my work with such acetates that the oxide deposited 130

by the same in the skin is very much more stable and gives a leather of great durability probably for the reason that during the tanning process the greatest part of the acetic acid is volatilized and that the oxide which is formed contains none or only very little of the acetic acid so as to be practically free of acid. The oxide thus deposited by this process in the skin is inert and shows no inclination to become either oxidized to a higher state of oxidation or to be reduced because there is no acid present to favor the transition of the oxide into a higher or lower state of oxidation as undoubtedly occurs with a great deteriorating effect on the hide treated with a solution containing cerium chloride.

For the reason that the atomic weights of the rare earth metals are very high as compared with that of aluminum, a greater quantity of the same will combine with the animal tissue and will therefore give the leather a greater whiteness than can be accomplished with compounds of lower atomic weight. As the quantity of acid in the molecule of the rare earth metal compounds is proportionately smaller than in the compounds of metals of low atomic weight, the amount of acid to produce the neutral salt, or the amount of alkali to turn such a salt into a basic salt is less, regardless of whether the salt be a sulfate, chloride or acetate, and the cost of the materials to perform these changes is smaller than with the other chemicals applied up to now as tanning agents. Moreover, as the compounds used in connection with my new tanning process are produced preferably from the waste products obtained in the manufacture of the salts for the impregnation of mantles for incandescent gas light, this fact in combination with the favorable circumstances pointed out above make it selfevident that my new tanning process can successfully compete as to economy as well as quality of products with any of the old tanning processes working even with such apparently low priced materials as alum.

Though in the far greater majority of cases my new tanning process will be applied to hides dehaired and bated in the usual ways I wish to state that my new invention can just as well be applied to pelts preserved in their natural hair cover. In the preparation of furs the pelts are usually wetted on the flesh-side with a solution of sulfuric acid and sodium chloride and are subsequently worked with butter and sawdust whereby soft furs are obtained which, however, present little resistance to moisture and heat. I have now found that wetting a pelt on the flesh side with a solution of acetates of rare earth metals, including cerium, yields a soft and better keeping fur, especially if the fur after the treatment with

the above mentioned rare earth metal acetates is finished by working it with fats, oils, or butter and sawdust.

I wish furthermore to state that the rare earth metal compounds in the leather as well as in the fur act as a mordant to the fiber and that the material treated with same can be dyed with a great variety of shades, giving to the leather a bright and rich appearance and to the furs the much desired lustre.

What I claim is:

1. The process of treating animal tissue, comprising acting in the presence of sodium chloride upon the tissue, prepared in any of the well known ways, with a solution of a salt of a rare earth metal capable of forming a basic salt.

2. The process of treating animal tissue, comprising acting in the presence of sodium chloride upon the tissue, prepared in any of the well known ways, with a solution of a salt formed by a volatile acid with any of the rare earth metals.

3. The process of treating animal tissue, comprising acting in the presence of sodium chloride upon the tissue, prepared in any of the well known ways, with a solution of an acetate of any of the rare earth metals.

4. The process of treating animal tissue, comprising acting in the presence of sodium chloride upon the tissue, prepared in any of the well known ways, with a solution of a basic acetate of any of the rare earth metals.

5. The process of treating animal tissue, comprising acting upon the tissue, prepared in any of the well known ways, in the presence of sodium chloride with a solution of the salts of a plurality of rare earth metals capable of forming basic salts.

6. The process of treating animal tissue, comprising acting upon the tissue, prepared in any of the well known ways, with a 10% solution of sodium chloride and a 5% solution of the basic acetates of rare earth metals.

7. The process of treating animal tissue, comprising acting upon the tissue, prepared in any of the usual ways, with a solution of acetates of the rare earth metals in the presence of egg-yolk, flour and sodium chloride.

8. The process of treating animal tissue, comprising acting upon the tissue, prepared in any of the usual ways, at approximately 37 deg. C. with a solution of acetates of the rare earth metals in the presence of egg-yolk, flour and sodium chloride.

9. The process of treating animal tissue, comprising acting at the flesh side of the tissue by wetting same with a solution of sodium chloride and a salt of rare earth metal.

10. The process of treating animal tissue, comprising acting at the flesh side of the tissue by wetting same with a solution of sodium chloride and an acetate of a rare earth metal, and then working the tissue thus

4  
treated with a fat and a vegetable mass like  
saw-dust.

11. As a new article of manufacture, a  
leather being substantially free of acid and  
5 having an oxide of a rare earth metal depos-  
ited in an inert state in its tissue.

12. As a new article of manufacture, a  
leather being substantially free of acid and  
10 having a mixture of inert oxides of rare  
earth metals deposited in its tissue.

13. The process of sterilizing hides, com-  
prising acting upon the raw hides, from  
which the flesh particles, or other organic  
matter, has been removed, with a solution of  
15 a salt of a rare earth metal capable of form-  
ing a basic salt.

14. The process of sterilizing hides, from  
which the flesh particles or other organic

matter has been removed, said process com-  
prising acting upon such hides in the pres-  
20 ence of sodium chloride with a solution of a  
salt of a rare earth metal capable of form-  
ing a basic salt.

15. The process of sterilizing hides, com-  
prising acting upon the raw hides, from  
25 which the flesh particles, or other organic  
matter, has been removed, with a solution of  
sodium chloride and a solution of the basic  
acetates of the rare earth metals.

16. The process of sterilizing hides, com-  
prising acting upon the raw hides, from  
30 which the flesh particles, or other organic  
matter, has been removed, with a solution of  
an acetate of a rare earth metal in the pres-  
ence of egg yolk, flour and sodium chloride.

FRIEDRICH WILHELM WEBER.